# EUROPEAN PATENT SPECIFICATION

(11) **EP 0 568 271 B1**
(45) Date of publication and mention of the grant of the patent: **19.06.1996**
(21) Application number: 93303148.6
(22) Date of filing: 22.04.1993
(51) Int. Cl.: D07B 1/06

(54) **Steel cords for reinforcement of rubber articles and pneumatic radial tires**
Stahlseile zur Verstärkung elastomerer Erzeugnisse und radialer Luftreifen
Câbles d'acier pour le renforcement des articles en caoutchouc et des bandages pneumatiques radiaux

(30) Priority: 27.04.1992 JP 107742/92
(43) Date of publication of application: 03.11.1993
(73) Proprietor: BRIDGESTONE CORPORATION, Tokyo 104 (JP)
(72) Inventor: Kuriya, Yoshinori, Kodaira City, Tokyo (JP)
(74) Representative: Whalley, Kevin

(56) References cited:
- EP-A- 0 373 595
- EP-A- 0 488 735
- GB-A- 720 149

## Description

This invention relates to steel cords used as a reinforcement for rubber articles such as pneumatic tires, industrial belts and the like as well as a pneumatic radial tire comprising a carcass ply comprised of such steel cords and having improved durability.

As rubber articles reinforced with steel cords, tires are well-known. Among them, tires for trucks and buses or for light trucks generally comprise a carcass ply using cords of two or three layer construction.

It is usual that the tensile load of the steel cord lowers during the running of the tire because the sectional area of steel filaments constituting the steel cord is decreased by fretting. In this case, if the decrease of sectional area in some filaments constituting the steel cord becomes conspicuous, such filaments are apt to undergo breakage as a result of tensile shock or repetitive bending. Once these filaments are broken, tensile stress in the other filaments increases to promote fatigue breakage of the cord. Therefore, in order to increase the durability of the cord, it is required to avoid a part of the steel filaments constituting the steel cord becoming prematurely broken as compared with the remaining steel filaments, and it is desirable that the tensile loads of all filaments in the cord are equally lowered.

Attention is drawn to the disclosure of EP-A-0 373 593, in particular to the prior art cords shown in figures 5 and 6 thereof.

It is an aim of the present invention to improve the durability of steel cords by equally lowering the tensile loads of the steel filaments in the steel cord due to decrease of filament sectional area through fretting during running when the steel cords are applied to a rubber article, particularly the carcass ply of the radial tire for trucks and buses.

The present inventor has made studies with respect to steel cords formed by spirally winding a wrap steel filament around a steel cord of layer twisting structure for stably preventing the lowering of tensile load in the steel filaments (filament diameter: 0.15-0.25 mm) constituting the steel cord used in a carcass ply during the running of a tire, and found that the lowering of tensile load in the steel filaments constituting the outermost layer of the steel cord is extremely large and that a main factor in the lowering of tensile load is a fretting phenomenon with the wrap filament.

Furthermore, the inventor has made studies with respect to steel cords formed by removing the wrap filament, which is the main factor in the lowering of tensile load, for preventing the occurrence of fretting around the wrap filament, and confirmed that the fretting is certainly removed to control the lowering of tensile load of the steel filament, but the restraining property of the cord is poor due to the absence of the wrap filament and furthermore when the cord is excessively bent, the steel filaments constituting the cord are scattered and finally broken when abnormal force is applied to the steel filaments. In the latter case, the life at break of the cord is largely decreased as compared with the cord stabilized by wrapping the cord with the wrap filament. As a result, in order to prevent the decrease of the cord life based on the application of extreme bending force, it becomes required to restrain the cord with the steel filament in any form.

Under the above circumstances, the inventor has made further studies with respect to the steel cord of layer twisting structure and discovered that it is advantageous to prevent the lowering of tensile load in the steel filaments of the outermost layer by controlling the application of abnormal force to the steel filament while maintaining the restraint of the filaments constituting the cord when a large bending force is applied to the cord and mitigating the fretting between the wrap filament and the steel filaments constituting the outermost layer of the cord, and as a result the invention has been accomplished.

According to a first aspect of the invention, there is provided a steel cord for the reinforcement of rubber articles formed by twisting 1 to 4 steel filaments as a core and at least one sheath layer comprised of a plurality of steel filaments arranged around the core, provided that the twisting pitch of at least one sheath layer is different from that of a remaining sheath layer adjacent thereto or that of the core, and wherein wrap steel filament is spirally wound around a sheath layer located at an outermost side of the steel cord in the same twisting direction as in one said sheath layer.

According to a second aspect of the invention, there is provided a pneumatic radial tire comprising a carcass ply of a radial structure toroidally extending between a pair of bead portions and containing steel cords therein, said steel cord being formed by twisting 1 to 4 steel filaments as a core and at least one sheath layer comprised of a plurality of steel filaments arranged around the core, provided that the twisting pitch of at least one sheath layer is different from that of a remaining sheath layer adjacent thereto or that of the core, and wherein a wrap steel filament is spirally wound around a sheath layer located at an outermost side of the steel cord in the same twisting direction as in the said sheath layer.

In a preferred embodiment of the invention, the wrap steel filament is wound around the outermost sheath layer at a twisting pitch of 2-6 mm. When the steel cords according to the invention are applied to the carcass ply of a pneumatic radial tire, the resistance to corrosion fatigue is improved and also the lowering of tensile load of the cord due to fretting between the outermost sheath layer and the wrap steel filament can be controlled while maintaining the restraint of the steel filaments in the cord.

The invention will be further described with reference to the accompanying drawings, wherein:
Fig. 1 is a diagrammatically sectional view of a steel cord having a layer twisting structure of 3+9+1;
Fig. 2 is a diagrammatically sectional view of a steel cord having a layer twisting structure of 1+6+12+1;
Fig. 3 is a diagrammatically sectional view of a steel cord having a layer twisting structure of 3+9+15+1; and
Fig. 4 is a schematic view illustrating a fretting depth h.

In Figs. 1 and 2 are sectionally shown embodiments of steel cord for the reinforcement of rubber articles according to the invention having layer twisting structures of 3+9+1 and 1+6+12+1, respectively. In Figs. 1 and 2, numeral 1 is a core comprised of one or three steel filaments, while numeral 2 is a sheath layer comprised of a plurality of steel filaments arranged adjacent to each other around the core 1. The sheath layer 2 is comprised of nine steel filaments in Fig. 1 and six steel filaments in Fig. 2. Further, a second sheath layer 3 comprised of twelve steel filaments is arranged around the sheath layer 2 in the embodiment of Fig. 2. In Figs. 1 and 2, numeral 4 is a wrap steel filament spirally wound around the outermost sheath layer in the same twisting direction as in the outermost sheath layer.

In Fig. 3 is sectionally shown a third embodiment of the steel cord according to the invention having a layer twisting structure of 3+9+15+1, in which a second sheath layer 3 comprised of 15 steel filaments is arranged around a first sheath layer 2 comprised of 9 steel filaments. As a modification of this embodiment, there may be used a steel cord having a layer twisting structure of 3+8+13+1.

In the conventional layer-twisted steel cord, the non-uniform lowering of tensile load in the steel filaments, particularly lowering of tensile load in the steel filaments of the outermost sheath layer, is due to the fact that the wrap steel filament is twisted in the direction opposite to the twisting direction of the steel filaments in the outermost sheath layer. Since the twisting direction of the wrap steel filament is different from that of the steel filaments in the outermost sheath layer, the contact area therebetween becomes small and the contact pressure per unit area is large.

During the running of a tire, torsion is applied to the carcass ply cord at a ground contact portion of the tire in the axial direction of the cord. When the torsional force is applied in a direction opposite to the twisting direction of the steel filaments in the outermost sheath layer, if the twisting direction of the wrap steel filament is opposite to the twisting direction of the steel filaments in the outermost sheath layer, torsional force is created in a direction of tightening the twisting direction of the wrap steel filament and hence a relative movement between the wrap steel filament and the steel filaments in the outermost sheath layer occurs. Therefore, when such a relative movement is caused under a large contact pressure, the reduction of sectional area in the steel filaments of the outermost sheath layer is promoted by the wrap steel filament and hence the tensile load of the steel filaments in the outermost sheath layer lowers.

According to the invention, the twisting direction of the spiral wrap steel filament restraining the steel cord of layer twisting structure is made in the same direction as the steel filaments of the outermost sheath layer, whereby the contact area between the steel filaments in the outermost sheath layer and the wrap steel filament is increased and the contact pressure therebetween is decreased. Further, even if torsional force is applied to the cord, the relative movement between the steel filaments in the outermost sheath layer and the wrap steel filament reduces and hence the reduction of sectional area in the steel filaments of the outermost sheath layer and the lowering of tensile load accompanied therewith are controlled. Moreover, since the steel filaments are restrained by the wrap steel filament, even when the cord is extremely bent, the steel filaments constituting the cord are not scattered and hence the breaking life of the cord is not lowered even when abnormal force is applied to a part of the steel filaments.

If the twisting direction is the same between the spiral wrap steel filament and the steel filaments in the outermost sheath layer, the filament diameter may be the same or different between the core and the sheath. On the other hand, if the twisting pitch of the steel filaments in the outermost sheath layer is the same as that of the spiral wrap steel filament, there is caused movement of the wrap steel filament into the outermost sheath layer, so that it is necessary that the twisting pitch of the steel filaments in the outermost sheath layer is different from that of the wrap steel filament.

Moreover, it is possible to wind the wrap steel filament in the same twisting direction as in the steel filaments of the outermost sheath layer by properly controlling the preforming ratio and torsion (residual torsional stress) of the wrap steel filament without obstructing the operability (curling after the cutting).

It is particularly preferable to apply the invention to a steel cord having a layer twisting structure of 3+8+1 in view of the cord durability. That is, when the invention is applied to rubber penetration type cords having a gap between the steel filaments in the sheath layer, if a large bending force is applied to the cord under a low internal pressure, the movement of the steel filaments becomes small because rubber penetrates into the inside of the cord and hence the resistance to cord breaking-up is improved.

The following examples are given in illustration of the invention and are not intended as limitations thereof.

### Example 1

Steel cords are prepared as shown in Table 1 and applied to a carcass ply of a radial tire for trucks and buses having a tire size of 11/70R22.5 14PR at an end count of 22.0 cords/5 cm. The fretting depth and cord breakage under large bending force are measured by running such a tire on a drum under the following test conditions:
- Speed:: 60 km/hr
- Internal pressure:: 8 kgf/cm² (usual running)
1 kgf/cm² (running under large bending force)
- Load:: JIS 100% load (usual running)
JIS 40% load (running under large bending force)

As the steel cord, there are used steel cord of Comparative Example 1 having a layer twisting structure of 3+9+1 and a wrap steel filament of Z-lay (control), steel cord of Comparative Example 2 having a layer twisting structure of 3+9 and no wrap steel filament, and steel cord of Example 1 having a layer twisting structure of 3+9+1 and a wrap steel filament of S-lay according to the invention. The measured results are shown in Table 1.

### Evaluation methods

### (1) Fretting depth

The steel filaments of the outermost sheath layer corresponding to two cords are taken out from the tire after the running under usual conditions and broken through a tensile test. Then, the broken sections of these filaments are observed by means of a microscope to measure a fretting depth h shown in Fig. 4 when the section of the original steel filament is circle. When an average of the measured values h is a fretting depth of the cord, the fretting depth is evaluated by an index value according to the following equation:
- Index =: fretting depth of test tire/ fretting depth of control x 100

### (2) Cord breakage under large bending force

The presence or absence of cord breakage is measured by taking out the steel cords from the tire after the running over a distance of 10,000 km under the large bending force.

**Table 1**

| | Comparative Example 1 | Comparative Example 2 | Example 1 |
|---|---|---|---|
| Twisting structure | 3+9+1 | 3+9 | 3+9+1 |
| Twisting direction | S/S/Z | S/S | S/S/S |
| Twisting pitch | 6.0/12.0/3.5 | 6.0/12.0 | 6.0/12.0/3.5 |
| Filament diameter (mm) | | | |
| (1) core, sheath | 0.23 | 0.23 | 0.23 |
| (2) wrap | 0.15 | - | 0.15 |
| Fretting depth | 100 | - | 8 |
| Cord breakage | none * | presence | none * |

| | | | |
|---|---|---|---|
| * : no filament breakage | | | |

### Example 2

Steel cords are prepared as shown in Table 2 and applied to a carcass ply of a radial tire for trucks and buses having a tire size of 11/70R22.5 14PR at an end count of 20.0 cords/5 cm. The fretting depth and cord breakage under large bending force are measured in the same manner as in Example 1 by running such a tire on a drum under the same conditions as in Example 1.

As the steel cord, there are used steel cord of Comparative Example 3 having a layer twisting structure of 1+6+12+1 and a wrap steel filament of Z-lay (control), steel cord of Comparative Example 4 having a layer twisting structure of 1+6+12 and no wrap steel filament, and steel cord of Example 2 having a layer twisting structure of 1+6+12+1 and a wrap steel filament of S-lay according to the invention. The measured results are shown in Table 2. Moreover, when the core is comprised of a single steel filament, the twisting pitch of the core is considered to be infinite.

**Table 2**

| | Comparative Example 3 | Comparative Example 4 | Example 2 |
|---|---|---|---|
| Twisting structure | 1+6+12+1 | 1+6+12 | 1+6+12+1 |
| Twisting direction | -/S/S/Z | -/S/S | -/S/S/S |
| Twisting pitch | ∞/6.0/12.0/3.5 | ∞/6.0/12.0 | ∞/6.0/12.0/3.5 |
| Filament diameter (mm) | | | |
| (1) core, sheath | 0.20 | 0.20 | 0.20 |
| (2) wrap | 0.15 | - | 0.15 |
| Fretting depth | 100 | - | 13 |
| Cord breakage | none * | presence | none * |

| | | | |
|---|---|---|---|
| * : no filament breakage | | | |

### Example 3

Steel cords are prepared as shown in Table 3 and applied to a carcass ply of a radial tire for trucks and buses having a tire size of 11/70R22.5 14PR at an end count of 19.8 cords/5 cm. The fretting depth and cord breakage under large bending force are measured in the same manner as in Example 1 by running such a tire on a drum under the same conditions as in Example 1.

As the steel cord, there are used steel cord of Comparative Example 5 having a layer twisting structure of 3+9+15+1 and a wrap steel filament of S-lay (control), steel cord of Comparative Example 6 having a layer twisting structure of 3+9+15 and no wrap steel filament, and steel cord of Example 3 having a layer twisting structure of 3+9+15+1 and a wrap steel filament of Z-lay according to the invention. The measured results are shown in Table 3.

**Table 3**

| | Comparative Example 5 | Comparative Example 6 | Example 3 |
|---|---|---|---|
| Twisting structure | 3+9+15+1 | 3+9+15 | 3+9+15+1 |
| Twisting direction | S/S/Z/S | S/S/Z | S/S/Z/Z |
| Twisting pitch | 5.5/10.5/15.5/3.5 | 5.5/10.5/15.5 | 5.5/10.5/15.5/3.5 |
| Filament diameter (mm) | | | |
| (1) core, sheath | 0.175 | 0.175 | 0.175 |
| (2) wrap | 0.15 | - | 0.15 |
| Fretting depth | 100 | - | 17 |
| Cord breakage | none * | presence | none * |

| | | | |
|---|---|---|---|
| * : no filament breakage | | | |

### Example 4

Steel cords are prepared as shown in Table 4 and applied to a carcass ply of a radial tire for trucks and buses having a tire size of 11/70R22.5 14PR at an end count of 31.8 cords/5 cm. The fretting depth and cord breakage under large bending force are measured in the same manner as in Example 1 by running such a tire on a drum under the same conditions as in Example 1.

As the steel cord, there are used steel cord of Comparative Example 7 having a layer twisting structure of 3+8+1 and a wrap steel filament of Z-lay (control), steel cord of Comparative Example 8 having a layer twisting structure of 3+8 and no wrap steel filament, and steel cord of Example 4 having a layer twisting structure of 3+8+1 and a wrap steel filament of S-lay according to the invention. The measured results are shown in Table 4.

**Table 4**

| | Comparative Example 7 | Comparative Example 8 | Example 4 |
|---|---|---|---|
| Twisting structure | 3+8+1 | 3+8 | 3+8+1 |
| Twisting direction | S/S/Z | S/S | S/S/S |
| Twisting pitch | 5.5/10.5/3.5 | 5.5/10.5 | 5.5/10.5/3.5 |
| Filament diameter (mm) | | | |
| (1) core, sheath | 0.21 | 0.21 | 0.21 |
| (2) wrap | 0.15 | 0.15 | 0.15 |
| Fretting depth | 100 | - | 8 |
| Cord breakage | none * | presence | none * |

| | | | |
|---|---|---|---|
| * : no filament breakage | | | |

As mentioned above, the steel cord according to the invention has such a layer twisting structure that the wrap steel filament is spirally wound around the outermost sheath layer in the same direction as in the steel filaments of the outermost sheath layer. When such steel cords are applied to the carcass ply of a radial tire, the fretting between the steel filaments of the outermost sheath layer and the wrap steel filament is decreased and also the lowering of tensile load in the steel filaments of the cord becomes equal to improve the cord life, so that the tire durability can considerably be improved.

## Claims

1. A steel cord for the reinforcement of rubber articles formed by twisting 1 to 4 steel filaments as a core (1) and at least one sheath layer (2,3) comprised of a plurality of steel filaments arranged around the core, provided that the twisting pitch of at least one sheath layer is different from that of a remaining sheath layer adjacent thereto or that of the core, and wherein a wrap steel filament (4) is spirally wound around a sheath layer located at an outermost side of the steel cord, characterized in that said wrap steel filament (4) is wound in the same twisting direction as in the said sheath layer.

2. A steel cord as claimed in claim 1, characterized in that said wrap steel filament (4) is wound around said outermost sheath layer at a twisting pitch of 2-6 mm.

3. A steel cord as claimed in claim 1 or 2, characterized in that said cord has a layer twisting structure selected from 3+9+1, 3+8+1, 1+6+12+1 and 3+9+15+1 types.

4. A pneumatic radial tire comprising a carcass ply of a radial structure toroidally extending between a pair of bead portions and containing steel cords therein, characterized in that said steel cord is as claimed in any of claims 1 to 3.

## Patentansprüche

1. Stahlcordfaden zur Verstärkung von Gummierzeugnissen, aus einer Seele (1), die durch Verdrillen von 1 bis 4 Stahlfilamenten gebildet wurde, und mindestens einer Mantelschicht (2, 3), die aus einer Vielzahl von um die Seele herum angeordneten Stahlfilamenten besteht, wobei die Verdrillsteigung von mindestens einer Mantelschicht verschieden von der Verdrillsteigung einer daran angrenzenden, verbleibenden Mantel schicht oder der Verdrillsteigung der Seele ist, und wobei ein Wickelstahlfilament (4) spiralförmig um die äußerste Mantelschicht des Stahlcordfadens herumgewickelt ist, dadurch gekennzeichnet, daß das Wickelstahlfilament (4) in der gleichen Verdrillrichtung wie diese äußerste Mantel schicht gewickelt ist.

2. Stahlcordfaden gemäß Anspruch 1, dadurch gekennzeichnet, daß das Wickelstahlfilament (4) mit einer Verdrillsteigung von 2-6 mm um die äußerste Mantelschicht herumgewickelt ist.

3. Stahlcordfaden gemäß Anspruch 1 oder 2, dadurch gekennzeichnet, daß der Cordfaden eine Schichtverdrillstruktur hat, die aus den Typen 3+9+1, 3+8+1, 1+6+12+1 und 3+9+15+1 ausgewählt ist.

4. Radialer Luftreifen, der eine Karkassenlage mit radialer Struktur aufweist, die sich toroidförmig zwischen zwei Wulstbereichen erstreckt und Stahlcordfäden enthält, dadurch gekennzeichnet, daß der Stahlcordfaden ein Stahl cordfaden ist, wie er in irgendeinem der Ansprüche 1 bis 3 beansprucht wird.

## Revendications

1. Câblé en acier pour le renforcement d'articles en caoutchouc, formé en torsadant de 1 à 4 filaments en acier comme partie centrale (1) et d'au moins une couche de gainage (2, 3) comprenant plusieurs filaments en acier arrangés autour de la partie centrale, dans lequel le pas de torsion d'au moins une couche de gainage est différent de celui d'une couche de gainage restante adjacente à la première ou de celui de la partie centrale, et dans lequel un filament d'enroulement en acier (4) est enroulé en spirale autour d'une couche de gainage située du côté le plus externe de câblé en acier, caractérisé en ce que ledit filament d'enroulement en acier (4) est enroulé dans la même direction de torsion que ladite couche de gainage.

2. Câblé en acier selon la revendication 1, caractérisé en ce que ledit filament d'enroulement en acier (4) est enroulé autour de ladite couche de gainage la plus externe à un pas de torsion de 2-6 mm.

3. Câblé en acier selon la revendication 1 ou 2, caractérisé en ce que ledit câblé possède une structure de torsion en couches choisie parmi les types 3+9+1, 3+8+1, 1+6+12+1 et 3+9+15+1.

4. Bandage pneumatique radial comprenant une nappe de carcasse de structure radiale s'étendant en forme toroïdale entre une paire de portions de talons et contenant des câblés en acier, caractérisé en ce que ledit câblé en acier est tel que revendiqué dans l'une quelconque des revendications 1 à 3.
